

July 21, 1959

R. W. FRITTS ET AL

2,896,005

THERMOELECTRIC HEAT PUMP

Filed June 1, 1955

5 Sheets-Sheet 1



INVENTORS.  
Robert W. Fritts,  
BY Sebastian Karrer,  
Brown, Johnson, Batteland & Dunn  
*Atttys.*

July 21, 1959

R. W. FRITTS ET AL

2,896,005

THERMOELECTRIC HEAT PUMP

Filed June 1, 1955

5 Sheets-Sheet 2

Fig. 3.



INVENTORS  
Robert W. Fritts,  
BY Sebastian Karrer,  
Norman J. Luhm, Fletcher L. Lunn  
C. F. Fritts

July 21, 1959

R. W. FRITTS ET AL

2,896,005

THERMOELECTRIC HEAT PUMP

Filed June 1, 1955

5 Sheets-Sheet 3

Fig. 5.



Fig. 5A.

INVENTORS.

Robert W. Fritts,  
BY Sebastian Karrer,  
Brown, Juhim, Botteler & Birren  
Atty's.

July 21, 1959

R. W. FRITTS ET AL

2,896,005

THERMOELECTRIC HEAT PUMP

Filed June 1, 1955

5 Sheets-Sheet 4

Fig. 6.



INVENTORS.  
Robert W. Fritts,  
BY Sebastian Karrer,  
Brown, Fidell, Bittner & Seinen  
Attn: S.

July 21, 1959

R. W. FRITTS ET AL

2,896,005

THERMOELECTRIC HEAT PUMP

Filed June 1, 1955

5 Sheets-Sheet 5

Fig. 7



INVENTORS.

Robert W. Fritts  
BY Sebastian Karre,  
Brown, Fidler, Bottcher & Seiner  
Otto S.

2,896,005

## THERMOELECTRIC HEAT PUMP

Robert W. Fritts, Elm Grove, Wis., and Sebastian Karrer, Port Republic, Md., assignors, by mesne assignments, to Minnesota Mining and Manufacturing Company, St. Paul, Minn., a corporation of Delaware.

Application June 1, 1955, Serial No. 512,436

13 Claims. (Cl. 136—5)

The present application is a continuation-in-part of our application, Serial No. 475,544, filed December 15, 1954, now abandoned, for Thermoelectric Heat Pump.

This invention relates to heat pumps and, more particularly, to heat pumps comprising single or multiple junctions of different thermoelectric elements.

A primary object of the invention is to provide thermoelectric heat pumps affording a rate of heat transfer and temperature differentials sufficiently high for practical use.

Another object is to provide heat pumps of the character aforescribed affording high efficiency and performance factors.

Another object is to provide thermoelectric heat pumps having at least one improved thermoelectric element which when connected in circuit with a source of direct current affords heat transfer through the thermoelectric element with resultant cooling of one portion and heating of another portion of the element in sufficient amount for practical use.

Another object is to provide heat pumps of the character aforescribed comprising thermoelectric elements of semimetallic compositions and more particularly certain binary and ternary compositions having semiconductor-like conductivity or conductance.

Other objects and advantages will hereinafter appear or will become apparent to those skilled in the art with reading of the following specification.

In the drawings:

Figure 1 is a somewhat schematic illustration of a single thermoelectric element heat pump embodying the invention;

Figure 2 is a somewhat schematic illustration of a compound or double thermoelectric element heat pump comprising thermoelectric elements of opposite polarity embodying the invention;

Figure 3 is a graphic illustration of certain lead-selenium-tellurium compositions comprising thermoelectric heat pump elements of the invention;

Figure 4 is a graphic illustration of certain lead-selenium-sulphur compositions comprising thermoelectric heat pump elements of the invention;

Figure 5 is a graphic illustration of certain electrical characteristics of negative thermoelectric heat pump elements embodying the invention;

Figure 5A is a graphic illustration of certain electrical characteristics of certain positive thermoelectric heat pump elements embodying the invention;

Figure 6 is a graphic illustration of the performance factors of heat pumps embodying the invention; and

Figure 7 is a graphic illustration of certain electrical characteristics of additional positive thermoelectric heat pump elements embodying the invention.

When a direct current is passed through a junction between two dissimilar conductors the junction is heated or cooled depending not only upon the direction of current flow but also upon the nature of the conductors. This heating or cooling of the junctions is called the Peltier effect and is linearly dependent upon the current

through the junction. The proportionality factor between heat absorption or evolution rate and electric current is called the Peltier coefficient and is equal to the heat transferred when unit quantity of electricity traverses the junction. The Peltier coefficient may be directly determined as the product of absolute temperature and the derivative with respect to temperature of the Seebeck E.M.F. Accompanying such effect under the circumstance stated is a transformation between thermal energy and electrical energy which takes place within each individual conductor, called the Thomson effect, which is defined as the heat absorbed or emitted per unit volume by a unit current passing through a unit temperature gradient. Such effects are reversible.

15 Metallic conductors, when joined to form a thermoelectric junction as aforescribed, exhibit low Peltier coefficients and low thermoelectric power. Moreover, such metallic conductors exhibit high thermal and electrical conductivity.

20 When an external voltage is introduced into the thermoelectric circuit, as aforementioned, the electric charges move according to the laws of conduction and as they pass the junctions of dissimilar conductors absorb or emit heat, thereby suffering a change in their electrostatic potential. This is called Peltier heat pumping, the Thomson effect being neglected since the temperature gradients within the thermoelectric elements are quite low in pumping.

25 In addition to the aforementioned reversible thermoelectric effects there are two other more common effects which must be considered in understanding the behavior of a thermoelectric heat pump. These are the conventional Joule heating, or  $I^2R$  dissipation (wherein  $I$  denotes current and  $R$  denotes resistance), and normal heat conductivity. In most applications of the Peltier heat pump these effects, which are irreversible, should be minimized for they are detrimental. Therefore, the resistivity and thermal conductivity of thermoelectric elements used in heat pumps should be as low as possible.

30 In Figure 1 the reversible Peltier effect is illustrated for a single thermoelectric element 10 conductively joined as at A and B to ordinary metallic conductors 11 and 12 completing a circuit to a source of direct current. The conductivity type of the thermoelectric element 10 is such that as unit current flows across junctions A and B,  $P_a$  units of heat are absorbed at junction A and  $P_b$  units of heat are emitted at B. The magnitudes of  $P_a$  and  $P_b$  depend upon the value of Peltier coefficient between the thermoelectric element 10 and the conductors 11 and 12 and upon the temperatures of the respective junctions. Where the junction temperatures are identical the heat absorbed at A equals the heat emitted at B.

35 If the initial temperature distribution in the pumping element is constant at  $T_0$ , then with time the absorption of heat by the current at "A" gradually lowers the junction temperature,  $T_a$ , and the emission at "B" gradually raises the temperature,  $T_b$ .

40 The extent to which  $T_a$  and  $T_b$  differ from  $T_0$  depends upon the magnitudes of the irreversible effects aforementioned as well as upon the magnitude of Peltier E.M.F.

45 The electrical energy input to the pumping element in the form of  $I^2R$  dissipation within the volume of the thermoelectric element raises the temperature of the thermoelectric element slightly. This irreversible input alters the temperature distribution within the thermoelectric element until it is balanced by an equal flow of heat out through the junctions. The other irreversible effect, heat conduction, causes a flow of heat from the high temperature region to the cooler portions; this is denominated as  $Q_c$ .

50 The establishment of temperature differences between the junctions and their external environments induces heat

flows therewith according to the laws of heat conduction; these are specified as  $Q_a$  and  $Q_b$ . When the current flow is held constant and the temperature distribution assumes a steady state then the total flow of heat into junction A equals the rate of Peltier absorption at junction A.  $(P_a = Q_a + Q_c + \frac{1}{2}I^2R)$ . Similarly, the flow of heat from junction B equals the rate of Peltier emission at junction B.  $(P_b = Q_b + Q_c - I^2R/2)$ .

As will be apparent, the important parameters for the operation of the pump are  $Q_a$ ,  $Q_b$ ,  $T_a$  and  $T_b$ .  $Q_a$  specifies the rate at which heat can be extracted from an external source in contact with the cooling junction A.  $Q_b$  specifies the rate at which heat can be delivered (exhausted) to an external source in contact with the heating junction B.  $T_b - T_a$  is the temperature difference through which the thermal energy is transferred. These parameters will be used henceforth in describing the performance of pumps; the other entities relating to phenomena occurring within the pumping element were specified merely to explain the pumping action and will not be mentioned further. It should be noted, however, that the difference between  $Q_a$  and  $Q_b$  is merely the electric power required to operate the pumping cycle.  $(Q_b - Q_a = EI = I^2R + Ide)$ . In the last, "de" is the differential thermal E.M.F. arising from the induced temperature difference  $T_b - T_a$ .

The direction of heat transfer of the thermoelectric element of Figure 1 is characteristic of elements having positive polarity of thermoelectric power and conductivity and with the current flowing in the direction indicated. For thermoelectric elements of negative polarity the heating and cooling of the junctions are just reversed. This is illustrated in Figure 2 wherein is shown a thermoelectric element 13 of positive polarity and a thermoelectric element 14 of negative polarity arranged in series circuit with respect to each other and a source of direct current. The arrow indicates the direction of electric current in the conventional sense—the electron flow is, of course, in the opposite direction. Accordingly, heating occurs at the junctions indicated as C and D between the thermoelectric elements 14 and 13 and electrical conductors 15 and 16, respectively, while cooling occurs at junctions designated E and F between thermoelectric elements 14 and 13 and a metallic conductor 17, respectively. In the arrangement shown in Figure 2, the heat transfer and consequent heating of junctions C and D and cooling of junctions E and F are additive, as will be apparent, thereby affording a heat pump of greater efficiency than one comprising a single thermoelectric element as shown in Figure 1. The heat pump of Figure 2 is, of course, possible only by virtue of utilization of thermoelectric elements 13 and 14 exhibiting Peltier E.M.F. and conductivity opposite in sign. The conductors, 15, 16 and 17 are metallic in composition and hence exhibit electrical and thermal properties characteristic of metals as aforementioned.

From the foregoing parameters we have derived an expression affording a convenient measure for comparison of thermoelectric elements and evaluation of their utility in heat pumps, which is hereinafter denominated the "Performance Factor" of the heat pump. This expression is  $\pi^2/2K\rho$  wherein

$\pi$  = Peltier coefficient

$K$  = Thermal conductivity

$\rho$  = Electrical resistivity

This expression is derived directly from an analysis of heat flow in thermoelectric heat pumps. The parameters involved are determined by conventional techniques and the term above (Performance Factor) is a measure of the capacity of the heat pump to create a temperature difference and convect heat through this difference.

The absorption or evolution of heat at a junction, as aforescribed, is directly proportional to  $\pi$ . The irreversible flow of heat down the temperature difference is proportional to  $K$  and the Joule ( $I^2R$ ) dissipation is proportional to  $\rho$ . The values of  $\pi$  and  $\rho$  are related through

the nature of the conduction processes in the compositions hereinafter described. From the foregoing expression it will be observed that the best heat pump will comprise thermoelectric elements having at one and the same time high values of Peltier E.M.F. ( $\pi$ ) and low values of thermal conduction ( $K$ ) and of resistivity ( $\rho$ ), or high conductivity.

The performance of thermoelectric heat pumps embodying this invention may also be stated in terms of the heating and cooling afforded at the junctions in relation to the amount of electrical energy required for such heating or cooling. An expression of this factor is denominated herein the "Performance Coefficient." The performance coefficient of a heat pump (with respect to the cooling junction) is defined as the ratio of heat absorbed at the cooling junction to the electrical energy dissipation within the pump and can be set forth as follows:

$$\frac{Q_a}{EI} = \frac{Q_a}{Q_b - Q_a}$$

20 The performance coefficient of a heat pump (with respect to the heating junction) is defined as the ratio of the heat exhausted at the heating junction to the electrical energy dissipation within the pump and can be set forth as follows:

$$\frac{Q_b}{EI} = \frac{Q_b}{Q_b - Q_a}$$

The performance coefficient of heating is equal to the performance coefficient for cooling plus one.

30 To provide heat pumps of high rate of heat transfer and high efficiency as aforementioned comprising one or more thermoelectric elements (as illustrated respectively in Figures 1 and 2), we have produced thermoelectric elements of new compositions exhibiting electrical characteristics as aforementioned superior for heat pumping purposes than known metallic alloys and thermoelectric elements of known semiconductive compositions.

We have found that certain alloys or intermetallic compounds exhibit very favorable relationships between 40 Peltier coefficient and resistivity and simultaneously favorable values of thermal conductivity. Further, we have found that the values of Peltier coefficient and resistivity may be arbitrarily and advantageously altered to afford a wide range of performance factors without significant 45 changes in thermal conductivity. Metals and metallic alloys exhibit low values of Peltier coefficient and resistivity and simultaneously high values of thermal conductivity. On the other hand, semiconductors exhibit low values of thermal conductivity and high values of 50 Peltier coefficient and resistivity. Performance factors for metals are low because of the high values of thermal conductivity. Performance factors for semiconductors are low because of their high resistivities. Our invention is based on the fact that we have found a way to alter the 55 electrical properties of certain intermetallic compounds (which in a pure state exhibit high Peltier coefficient and resistivity and low values of thermal conductivity) to reduce their resistivity without a proportionate reduction in Peltier coefficient or a significant increase in thermal 60 conductivity. These intermetallic compounds, which in a pure state are semiconductors, are altered by adding small concentration of beneficial impurity which render the semiconductors somewhat more metallic in nature, thereby vastly improving the performance factor. The 65 resulting compositions exhibit high values of Peltier coefficient and low values of resistivity and thermal conductivity in a relationship which cannot be achieved in either pure metals or pure semiconductors. Such resulting compositions we have denominated "semi-metallic" 70 alloys or compositions (to distinguish them from metallic alloys on the one hand and semiconductor alloys on the other hand). Such semi-metallic alloys or compositions for the first time afford Peltier heat pumping with induced temperature differences and pumping rates of sufficient 75 magnitude for utilization in practical applications.

The semi-metallic alloys or compositions aforementioned may, we have found, be characterized as binary metallic compounds of slightly imperfect composition, i.e. containing beneficial impurities constituting departures from perfect stoichiometry by reason of an excess of one of the metals over the other, and/or containing added beneficial impurity substances denominated hereinafter "promoters." Such semi-metallic compositions have semiconductor-like conductance (both electrical and thermal, as aforementioned). Semi-metallic alloys or compositions also include mixtures of such binary metallic compounds, which may be denominated ternary metallic alloys or compositions.

More specifically, we have found especially useful for heat pumping thermoelectric elements comprising lead and at least one member of the group tellurium, selenium and sulphur in proportions hereinafter described and to which may be added beneficial impurity substances in the form of promoters, as will also hereinafter be described. As will appear, certain of these alloys or compositions exhibit negative and certain exhibit positive electrical characteristics thereby affording, if desired, a compound or double heat pump unit as shown in Figure 2.

Referring now to Figure 3, there are graphically illustrated therein a multiplicity of examples of semi-metallic compositions or alloys for thermoelectric heat pump elements comprising lead and tellurium or selenium. It will be observed that the horizontal coordinate of this graph represents the various proportions of tellurium and selenium given in atomic percent and ranging linearly from tellurium containing but a "trace" (as hereinafter defined) of selenium on the left to selenium containing but a "trace" of tellurium on the right. The left-hand vertical scale (in terms of percent by weight) gives the amount of lead which can be alloyed with the tellurium, selenium or tellurium-selenium constituent for any proportions of the latter while the right-hand vertical scale conversely gives the percent by weight of the tellurium, selenium or selenium-tellurium constituent for any proportions of the latter in the final composition, the remainder, of course, being lead.

Figure 3 graphically illustrates compositions or alloys comprising lead and either tellurium or selenium or both since, we have discovered, selenium and tellurium when alloyed with lead within the proportions indicated are mutually soluble throughout the range of compositions illustrated and that tellurium and selenium are interchangeable for purposes of providing suitable thermoelectric heat pump elements falling within the class of binary metallic compounds aforementioned, and due to such mutual solubility, such binary compounds of the constituents indicated may be mixed, as is also graphically illustrated, to provide the ternary alloys or compositions also hereinbefore mentioned. The discovery of such interchangeability of selenium and tellurium is important in the economic manufacture of thermoelectric elements of the character aforeindicated in that it eliminates the necessity for separating selenium from tellurium and vice versa (these two constituents being invariably found together as contaminants one to the other), a difficult and expensive procedure, and indeed impossible of complete achievement. Accordingly, even the end extremes of the compositions illustrated in Figure 3, i.e. that of the left-hand end of the scale (35.0% to 38.05% by weight tellurium, remainder substantially all lead) may be considered as containing at least a "trace" of selenium, while the composition at the other end of the scale (25.0% to 27.55% by weight selenium, remainder substantially all lead) may be considered as containing at least a "trace" of tellurium. Accordingly, where the term "trace" is used hereinafter in the specification and claims, it is to be understood as meaning amounts of the specified constituents and/or contaminants so small as to defy detection but which must be assumed to be present due to the impossibility of achieving absolute purity.

Again referring to Figure 3, by way of example, it will be observed that a thermoelectric element of lead, selenium and tellurium affording the desired characteristics could consist, as aforescribed, of a selenium-tellurium constituent in which the selenium is but a trace. In this case such constituent should constitute from 35.0% to 38.05% by weight of the composition, the balance (65.0% to 61.95% by weight) being lead. On the other extreme, where the selenium-tellurium constituent consists almost entirely of selenium, with but a trace of tellurium, such constituent should comprise from 25.0% to 27.55% by weight of the final composition, the remainder (from 75.0% to 72.45% by weight) being lead. These extreme compositions, aforescribed, may for purposes of this specification and claims be denominated "terminal" compositions and may be considered binary metallic compounds of slightly imperfect compositions as will hereinafter appear.

As a further example, where the selenium and tellurium are equal (in atomic percent) in the selenium-tellurium constituent, the latter should constitute from 30.0% to 32.8% by weight of the composition, the remainder (70.0% to 67.2% by weight) being lead. Such a composition, as well as all other compositions illustrated in Figure 3, intermediate the terminal compositions aforescribed, are mixtures (in various proportions) of the terminal compositions and since they contain both selenium and tellurium as well as lead, are ternary alloys or compositions.

Referring now to Figure 4 there are graphically illustrated therein a further multiplicity of examples of semi-metallic compositions or alloys for thermoelectric heat pump elements comprising lead and selenium or sulphur. As is the case in Figure 3, the horizontal coordinate of the graph of Figure 4 represents the various proportions of selenium and sulphur given in atomic percent and ranging linearly from selenium containing but a trace, as above defined, of sulphur on the left to sulphur containing but a trace of selenium on the right. The left-hand vertical scale (in terms of percent by weight) gives the amount of lead which can be alloyed with the selenium, sulphur or selenium-sulphur constituent for any proportions of the latter, while the right-hand vertical scale conversely gives the percent by weight of the sulphur, selenium, or selenium-sulphur constituent for any proportions of the latter in the final composition, the remainder, of course, being lead.

Figure 4 further graphically illustrates compositions or alloys comprising lead and either selenium or sulphur or both since, we have discovered, selenium and sulphur when alloyed with lead within the proportions indicated are mutually soluble throughout the range of compositions illustrated and that selenium and sulphur are interchangeable for purposes of providing suitable thermoelectric heat pump elements falling within the class of binary metallic compounds aforementioned, and due to such mutual solubility such binary compounds of the constituents indicated may be mixed as is also illustrated to provide the ternary alloys or compositions also hereinbefore mentioned. The discovery of such interchangeability of selenium and sulphur is important in the economic manufacture of thermoelectric elements of the character aforeindicated in that it eliminates the necessity for separating selenium from sulphur and vice versa (these two constituents being invariably found together as contaminants one to the other), a difficult and expensive procedure and indeed impossible of achievement. Accordingly, even the end extremes of the compositions illustrated in Figure 4, i.e. that of the left-hand end of the scale (25.0% to 27.55% by weight selenium, remainder lead) may be considered as containing at least a trace of sulphur, while the composition at the other end of the scale (12.80% to 13.37% by weight sulphur, remainder substantially all lead) may be considered as containing at least a trace of selenium.

Again referring to Figure 4, by way of example, it will be observed that a thermoelectric element of lead, selenium and sulphur affording the desired characteristics could consist, as aforescribed, of a selenium-sulphur constituent in which the sulphur is but a trace. In this case, such constituent should constitute from 25.0% to 27.55% by weight of the composition, the balance (75.0% to 72.45% by weight) being lead. On the other extreme, where the selenium-sulphur constituent consists almost entirely of sulphur with but a trace of selenium, such constituent should comprise from 12.80% to 13.37% by weight of the final composition, the remainder (87.20% to 86.63% by weight) being lead. These extreme compositions aforescribed may also, for purposes of the specification and claims, be denominated "terminal" compositions and may be considered binary metallic compounds of slightly imperfect composition as will hereinafter appear.

As a further example, where the selenium and sulphur are equal (in atomic percent) in the selenium-sulphur constituent, the latter should constitute from 18.90% to 20.46% by weight of the composition, the remainder (81.10% to 79.54% by weight) being lead. Such a composition, as well as other compositions illustrated in Figure 4 intermediate the terminal compositions aforescribed, are mixtures (in various proportions) of the terminal compositions and since they contain both selenium and sulphur as well as lead, are ternary alloys or compositions.

We have also discovered that the terminal compositions aforescribed consisting substantially entirely of lead and tellurium may to a limited extent contain some sulphur (i.e. to the extent that sulphur is found as a contaminant in commercially available tellurium) as well as selenium. Similarly, the terminal compositions aforescribed consisting substantially of lead and selenium may contain to a limited extent tellurium and sulphur, as the case may be, and the terminal compositions aforescribed consisting substantially of lead and sulphur may contain tellurium to a limited extent as aforescribed as well as selenium. Likewise any of the intermediate or ternary alloys or compositions consisting of lead and at least two members of the group tellurium, selenium, sulphur, may contain such limited amounts of the other element of the group.

The proportions and ranges of the various constituents aforescribed as illustrated in the graphic representation constituting Figures 3 and 4 of the drawings must be considered critical if the compositions illustrated are to have the electrical properties desired in heat pumps as aforescribed. The minimum limits of the lead constituent in the compositions of the invention (illustrated graphically by the lower curve in Figures 3 and 4) must be regarded as critical since if the lead content is significantly less than this amount for any particular proportions of the constituents, desired values of Peltier E.M.F. and resistivity will not be afforded and the significant electrical and mechanical properties will not be reproducible. On the other hand, if the lead content of any composition appreciably exceeds the maximum limit (illustrated graphically by the upper curve of Figures 3 and 4) the resulting composition, we have found, is too metallic in nature to afford electrical characteristics satisfying the objects of this invention.

Not only are the proportions and ranges aforescribed considered to be critical, but so also is the purity. More specifically, the limit of tolerable metallic impurity in the final composition has been found to be on the order of 0.01% and the composition must be substantially oxygen free if the mechanical and electrical properties desired are to be obtained and be reproducible. Such purity may be achieved by utilization of lead, tellurium, selenium and sulphur which do not contain metallic impurities exceeding the order of 0.01%. Alternatively, starting constituents of lesser purity may be utilized

where the formed composition is put through a recrystallization step, to be hereinafter described, to provide the final or end composition of the order of purity aforescribed. Accordingly, the starting ingredients or, in any event, the final composition where mentioned in this specification and appended claims are to be understood to be of the order of purity aforescribed. Several impurities commonly found in commercial stocks of all four of the constituents will reduce the Peltier E.M.F. exhibited by compositions of the present invention and hence must be substantially removed by purification. For example, copper is one example of such an impurity having a deleterious effect.

Compositions of lead and at least one of the group tellurium, selenium, sulphur, aforescribed, affording the desired electrical properties aforescribed may be produced by the following method. The starting constituents, free of metallic contaminants as aforescribed, and preferably in a reduced state, are mixed together in the proportions indicated hereinbefore and sealed in a tube or container preferably of quartz or Vycor, the container first being evacuated. The tube and its contents are then heated to the melting point of the latter which occurs at a temperature ranging from about 920° C. for the terminal compositions graphically illustrated at the left-hand extreme of Figure 3 to 1085° C. for the terminal compositions illustrated at the right-hand extreme of Figure 3 and the left-hand extreme of Figure 4, respectively, to 1115° C. for the terminal compositions illustrated at the right-hand extreme of Figure 4. The particular temperature for any given composition illustrated in Figures 3 and 4 depends upon the melting point of that composition which can readily be deduced by those skilled in the art from that of the terminal compositions given by way of example. During such heating the molten mass is preferably agitated to insure good mixing and then cooled.

After the composition has been formed as aforescribed, the solidified ingot can be removed from the tube and cast in molds of graphite or the like under an atmosphere of inert gas. More specifically, during casting we have found it preferable to cover the mold with an inert gas such as, for example, argon or carbon dioxide under positive pressure. This gas suppresses the vaporization rate of the molten composition, thereby reducing porosity of the casting.

The aforescribed alloying and casting steps should be carried out in crucibles which do not react with or contaminate the composition since, as aforescribed, minor amounts of undesired impurities may very deleteriously affect the electrical and/or physical properties of the element. Suitable crucibles are, we have found, those made of carbon, Alundum, pre-fired lavite and Vycor or quartz.

After casting the ingots may be machined if necessary. The shaped ingots are then preferably annealed in a reducing atmosphere at from 540° C. to 815° C. for from 20 to 10 hours. This annealing treatment insures homogeneity of the ingots and enhances its electrical and physical properties.

An alternate method of forming the composition comprises melting the constituents aforescribed in an open crucible under an atmosphere of argon or any inert and/reducing gas. Since the vapor pressure of selenium and sulphur are relatively high, some loss of selenium or sulphur may be encountered and adjustments in the initial amount of this constituent, where used, must be made to account for this loss. In all other respects this method is similar to that previously described.

Thermoelectric heat pump elements comprising alloys or compositions of the invention can be achieved as aforescribed through utilization of starting constituents of such purity that the compositions and resultant alloy contains no more impurity than that aforescribed.

Alternatively, an alloy of such purity may be afforded by forming the composition as to be hereinafter described from less pure starting constituents and reducing the impurity content by recrystallization from the melt. As will be understood by those skilled in the art, this comprises melting the impure composition and causing slow solidification thereof progressively from one end of the melt to the other. This results in concentration of the impurities of the starting constituents in the region of the last point of the melt to solidify, which region may then be discarded and after which the process may, if further purification is necessary, be repeated. Where this method of purification is employed a small amount of additional lead, must then be added in amount sufficient to bring the resultant composition within the limits aforeindicated.

The aforementioned alloys of lead and at least one of the group tellurium, selenium, sulphur, may be best described metallographically as two-phase alloys. It has been observed that these two-phase alloys, when sectioned and examined microscopically, comprise a major phase comprising crystal grains varying usually from 1 to 10 millimeters in size and between such grains there exist thin, relatively darker regions of a second phase. The grains of the primary phase are crystals of the intermetallic compounds lead-telluride, lead-selenide and lead-sulphide (or mixed crystals thereof), which contain approximately 61.89%, 72.41% and 86.60% lead by weight, respectively. The darker second phase, clearly discernible at the grain boundaries, is lead containing a minor concentration of selenium, tellurium or sulphur. The function of the second phase in such alloys is thought to be three fold. First, the thermal equilibrium between the two phases, which is established by the heat treatment aforementioned, induces negative Peltier E.M.F. and conductivity in the primary lead-telluride, lead-selenide or lead-sulphide phase which, because of its high concentration in the alloy, controls the electrical properties of the two-phase alloy. Secondly, the thin layers act as a cementing agent for the grains of the primary phase, thereby improving the mechanical strength of the alloy when compared with that of the pure intermetallic compound. Thirdly, this cementing action of the second phase affords good electrical conductivity in the polycrystalline alloy by rendering the intergranular component of electrical resistivity negligible. We have found that the actual concentration of second phase is not critical so long as the composition is maintained within the aforementioned specified ranges.

With regard to such aforementioned specified ranges for the various compositions aforementioned, it will be observed that in each case there is an excess of lead over and above the amount thereof necessary for satisfying the stoichiometric proportions of the compound formed with the second constituent or constituents, i.e. the tellurium, selenium or sulphur. Taking by way of example the aforementioned terminal compositions, it will be noted that the first terminal composition consisting substantially of lead and tellurium contains from 61.95% to 65.0% by weight lead, or from .16% to 8.9% lead by weight of the total composition over and above the 61.89% lead stoichiometrically necessary to combine with the tellurium. Similarly, the terminal composition consisting substantially of lead and selenium contains from .15% to 10.4% lead by weight of the total composition over and above the 72.41% by weight lead stoichiometrically necessary for combination with the selenium. The same is, of course, true with respect to the terminal composition consisting substantially of lead and sulphur wherein the amount of lead specified for composition of the present invention is from .23% to 4.7% lead by weight of the total composition more than that necessary to stoichiometrically combine with the sulphur present, i.e. 86.60% by weight lead. Similarly, for any of the compositions intermediate the aforementioned

terminal compositions there exists within the composition ranges specified in Figures 3 and 4 an excess of lead over and above that stoichiometrically necessary to combine with the tellurium-selenium or selenium-sulphur constituent in percent by weight varying according to the relationship of such intermediate composition to the terminal compositions.

The excess of lead aforementioned inherent in all of the compositions aforementioned within the ranges thereof graphically illustrated in Figures 3 and 4 may be denominated an impurity with respect to the primary lead-telluride, lead-selenide and lead-sulphide phases, as the case may be. Such impurities, however, must be distinguished from the undesired impurities discussed hereinbefore in connection with the required purity requirements of the compositions or alloys. Accordingly, for purposes of this specification and the appended claims such excess lead amounts purposely present in the compositions will be denominated "beneficial impurities." As aforementioned, it is the presence of such beneficial impurities that affords the compositions of this invention their desired electrical characteristics and distinguishes the semi-metallic alloys or compositions of this invention from the primary phase intermetallic compounds lead-telluride, lead-selenide and lead-sulphide. More specifically, such beneficial impurities afford such intermetallic compounds, whether the binary compounds of the terminal compositions or the ternary alloys of the intermediate compositions, a lower resistivity without proportional sacrifice of Peltier E.M.F. or low thermal conductivity and which results in a composition having what may be termed semiconductor-like electrical conductance or conductivity. It should be noted that such excess lead induces in each of the compositions aforementioned a Peltier E.M.F. of negative polarity and negative conductivity, thereby affording a thermoelectric heat pump element having utility in, for example, the single element heat pump of Figure 1 or in combination with a thermoelectric heat pump element of opposite polarity, the double or compound heat pump of Figure 2.

We have further discovered that the electrical characteristics desirable in thermoelectric elements for heat pump applications of the aforementioned lead-tellurium, lead-selenium, lead-tellurium-selenium, lead-sulphur and lead-selenium-sulphur compositions of the aforementioned range and purity (for convenience hereinafter denominated "base compositions") can be markedly and advantageously altered in a reproducible manner by the addition thereto of controlled amounts of matter other than the constituents of the base composition. Such additions may also be denominated "beneficial impurities" as distinguished from undesired impurities as aforementioned. For convenience, these additions are herein designated "promoters" since, as will hereinafter appear, they tend to enhance the electrical characteristics desired in thermoelectric heat pump elements of the base composition. Since, as will hereinafter appear, the amounts of such promoters in terms of percent by weight of the base composition are very small, for such promoters to be most effective and afford reproducibility of electrical properties the base composition to which they are added should be of even greater purity, i.e. contain even less of undesired and uncontrolled impurities. As a practical matter we have found that the base composition should be of such purity in this regard as to contain not in excess of 0.001% by weight undesired impurity. Similarly, where such promoters are added, the lead content of the base composition should be slightly less; e.g. a maximum of 63.0%, 73.5% and 87.10% by weight, respectively, for the various terminal compositions.

As has previously been observed, all of the aforementioned base compositions exhibit negative Peltier E.M.F. and negative conductivity. By the addition of the promoters to be hereinafter described such negative properties may be enhanced by the addition of certain promoters while the polarity of the electrical properties of the base

composition may be reversed by the addition of certain other promoters. Accordingly, certain promoters will be denominated "positive promoters" and certain others will be denominated "negative promoters," as hereinafter defined, and the resultant alloy or composition may be "positive" or "negative" alloy or composition, as also hereinafter defined.

"Negative" compositions or alloys are to be understood throughout this specification and appended claims as meaning an alloy or composition which exhibits negative conductivity as evidenced by Hall effect measurements or thermoelectric effect measurements, both taken at room temperature. Similarly, "positive" compositions or alloys are to be understood as meaning an alloy or composition which exhibits positive conductivity as evidenced by Hall effect measurements or thermoelectric effect measurements, both taken at room temperature.

"Negative promoters" are those which when added to the base alloys aforescribed alter the electrical conductivity thereof without changing the polarity of the conductivity or Peltier E.M.F. of the base alloys (it being negative according to the preceding definition). "Positive promoters" are those which when added in amounts hereinafter disclosed to the base alloys aforescribed and certain base alloys hereinafter disclosed are effective in enhancing the electrical conductivity in a positive sense as above defined with only slight decrease in the thermoelectric power of the promoted base alloy. Certain of such "positive promoters" when added to the base alloys aforescribed cause at first with very small additions reduction in the conductivity of the alloy to a minimum value beyond which further increase in the concentration of the "positive promoters" causes an increase in the conductivity of the alloy accompanied by a reversal in the polarity of the conductivity and Peltier E.M.F., i.e. from negative to positive.

The functions of such negative and positive promoters should be contrasted for the sake of clarity as follows:

(1) Increasing concentrations of the negative promoters cause increases in the conductivity and decrease of the Peltier E.M.F. of the resulting alloy as compared to that of the base alloy while preserving the negative polarity of the conductivity and Peltier E.M.F. thereof.

(2) Increasing concentrations of the positive promoters cause initially reductions in the conductivity and increase in the Peltier E.M.F. of the base alloy until a minimum conductivity is reached whereupon the Peltier E.M.F. and conductivity reverse polarity to the positive sense and further increase in the concentrations of the positive promoters causes increase in the conductivity and decrease in the Peltier E.M.F. in the resulting alloy.

The promoters which we have found effective for the purposes of the present invention when added in minor amounts to the base compositions aforescribed will for convenience be discussed in terms of the terminal compositions modified as to purity and lead content as aforescribed, it being understood that such promoters may also be added to any of the intermediate compositions with beneficial results. In this case the promoters added should be proportioned both in kind and in amount according to the relative concentrations of the terminal compositions in the intermediate composition comprising a mixture of such terminal compositions.

Table I below, first column thereof, lists the additions which we have found effective as negative promoters when added to the aforescribed lead-tellurium base alloys or compositions. The second column of Table I lists the order of the maximum concentration limits by weight percent of such promoters to the base alloys effective for achieving the objects of the invention. It is to be understood that these concentration limits are the maximum which effectively alter the electrical properties of the base alloy. Concentrations in excess of the stated amounts of such additives have no appreciable effect in beneficially altering the electrical properties with which

this invention is concerned, and in this sense the limits indicated are to be considered critical. The third and fourth columns of Table I set forth the electrical properties at room temperature of lead-tellurium alloys promoted with the maximum useful concentrations of the negative promoters after high temperature annealing as hereinbefore described.

Table I

| 10 | Negative promoters | Order of maximum effective concentration limits by weight percent, 0.80 | Peltier E.M.F., volts, 0.022 | Resistivity, ohm-cm., 0.00020 |
|----|--------------------|-------------------------------------------------------------------------|------------------------------|-------------------------------|
| 15 | Bismuth.....       | <sup>1</sup> 0.60-1.20                                                  | -0.022                       | 0.00031                       |
|    | Tantalum.....      | 0.50                                                                    | -0.036                       | 0.00032                       |
|    | Manganese.....     | 0.25                                                                    | -0.034                       | 0.00036                       |
|    | Zirconium.....     | 0.25                                                                    | -0.007                       | 0.00012                       |
| 20 | Titanium.....      | 0.15                                                                    | -0.014                       | 0.00020                       |
|    | Aluminum.....      | 0.10                                                                    | -0.018                       | 0.00016                       |
|    | Gallium.....       | 0.25                                                                    | -0.011                       | 0.00015                       |
|    | Chlorine.....      | 0.10                                                                    | -0.014                       | 0.00019                       |
| 25 | Bromine.....       | 0.20                                                                    | -0.014                       | 0.00015                       |
|    | Iodine.....        | 0.25                                                                    | -0.014                       | 0.00015                       |
|    | Uranium.....       |                                                                         |                              |                               |

<sup>1</sup> The range set forth is discussed below.

As previously mentioned, certain positive promoters may also be alloyed with the aforescribed lead-tellurium base alloys and such promoters are listed in column 1 of Table II. The second column of Table II like the corresponding column of Table I sets forth the order of the maximum concentration limits by weight percent of such promoters to the base alloys effective for achieving the objects of the invention. Again it will be observed that concentrations of the positive promoters to the lead-tellurium base alloys in amounts in excess of that contained in column 2 of Table II have no appreciable effect in beneficially altering the electrical properties with which this invention is concerned, and in this sense the limits indicated are to be considered critical.

Column 3 of Table II sets forth the minimum concentration by weight percent of the positive promoters listed affording useful heat pump elements of positive polarity.

Columns 4 and 5 set forth the Peltier E.M.F. and resistivity characteristics at room temperature of the alloy or composition resulting from the addition of the aforescribed positive promoters in the amount shown in column 2 after high temperature annealing as aforescribed.

Table II

| 55 | Positive promoters | Order of maximum effective concentration limit by weight percent | Order of minimum effective concentration limit by weight percent | Peltier E.M.F., volts | Resistivity, ohm-cm. |
|----|--------------------|------------------------------------------------------------------|------------------------------------------------------------------|-----------------------|----------------------|
| 60 | Sodium.....        | 0.06                                                             | 0.0008                                                           | +0.052                | 0.00074              |
|    | Potassium.....     | 0.10                                                             | 0.0009                                                           | +0.059                | 0.00076              |
|    | Thallium.....      | <sup>1</sup> 0.25-1.00                                           | <sup>1</sup> 0.01-0.04                                           | +0.077                | 0.0029               |
| 65 | Arsenic.....       | <sup>1</sup> 0.07-0.25                                           | <sup>1</sup> 0.002-0.006                                         | +0.081                | 0.0045               |

<sup>1</sup> The range set forth is discussed below.

As aforescribed, the lead-tellurium base alloy previously described is a two-phase alloy. When the aforescribed promoter additions are incorporated in the base alloy, such promoter additions become distributed between the two phases. We have discovered that the nature of such distribution has negligible effect on the electrical properties of the composition in all cases except that of bismuth, thallium and arsenic. Accordingly, in

the case of bismuth, thallium and arsenic the maximum effective concentration is dependent upon the lead content of the lead-tellurium base alloy within the ranges stated therefor as shown in Figure 3. We have found 1.20% by weight bismuth to be the maximum effective concentration for lead-tellurium base alloys containing 63.0% lead; for base alloys containing less lead the maximum effective bismuth concentration is somewhat less, that is ranges down to 0.60% by weight when the lead content ranges down to 61.95%. Similarly, in the case of thallium, the maximum effective concentration is dependent upon the lead content of the lead-tellurium base alloy within the range stated therefor. We have found 1.00% by weight thallium to be the maximum effective concentration for lead-tellurium base alloys containing 63.0% lead; for base alloys containing less lead the maximum effective thallium concentration is somewhat less, that is ranges down to 0.25% by weight when the lead content ranges down to 61.95%. Similarly, in the case of arsenic the maximum effective concentration is dependent upon the lead content of the lead-tellurium base alloy within the range stated therefor and ranges from 0.25% for base alloys containing 63.0% lead down to 0.07% for base alloys containing 61.95% lead. As indicated in Table II, the minimum effective concentration weight percent for heat pump elements in the case of thallium promoted base alloys ranges from 0.01% to 0.04% as the lead constituent of the lead-tellurium base composition varies from 61.95% to 63.0%. Similarly, in the case of the arsenic promoted base alloy the minimum effective concentration weight percent ranges from 0.002% to 0.006% as the lead content of the base alloy varies from 61.95% to 63.0%.

This behavior of bismuth, thallium and arsenic is thought to be due to the formation of a bismuth-lead-tellurium, thallium-lead-tellurium or an arsenic-lead-tellurium complex within the intergranular phase aforementioned which accounts for a portion of the addition. All other third element additions aforementioned, both positive and negative, form complexes with the second or intergranular phase aforementioned to a much lesser extent than do bismuth, thallium and arsenic and for purposes of this invention, in the cases of such other additions these effects are inconsequential. Accordingly, no changes in the concentration limits thereof are necessary as the proportions of lead and tellurium in the base alloy vary within the range stated therefor.

In Tables I and II above, the Peltier E.M.F. and resistivity data given is in both cases for the 61.95% lead, balance substantially all tellurium composition containing the promoter addition in question in the maximum effective amount indicated in the table (in the case of bismuth, thallium and arsenic, the lower maximum effective amount indicated).

Table III below, first column thereof, lists the additions which we have found effective as negative promoters when added to the aforementioned lead-selenium base alloys or compositions. The second column of Table III lists the order of the maximum concentration limits by weight percent of such promoters to the base alloys effective for achieving the objects of the invention. It is to be understood that these concentration limits are the maximum which effectively alter the electrical properties of the base alloy. Concentrations in excess of the stated amounts of such additives have no appreciable effect in beneficially altering the electrical properties with which this invention is concerned, and in this sense the limits indicated are to be considered critical. The third and fourth columns of Table III set forth the electrical properties at room temperature of lead-selenium alloys promoted with the maximum useful concentrations of the negative promoters after high temperature annealing as hereinbefore described.

Table III

|    | Negative promoters | Order of maximum effective concentration limits by weight percent | Peltier E.M.F., volts | Resistivity, ohm-cm. |
|----|--------------------|-------------------------------------------------------------------|-----------------------|----------------------|
| 5  |                    |                                                                   |                       |                      |
| 10 | Iodine             | 0.50                                                              | 0.012                 | 0.00016              |
|    | Chlorine           | 0.20                                                              | 0.011                 | 0.00018              |
|    | Zirconium          | 0.60                                                              | 0.008                 | 0.00016              |
|    | Bromine            | 0.60                                                              | 0.010                 | 0.00014              |
|    | Silicon            | 0.10                                                              | 0.016                 | 0.00024              |
|    | Titanium           | 0.10                                                              | 0.012                 | 0.00026              |
|    | Indium             | 0.20                                                              | 0.018                 | 0.00024              |
|    | Tantalum           | 0.60                                                              | 0.014                 | 0.00022              |
| 15 | Gallium            | 0.15                                                              | 0.017                 | 0.00027              |
|    | Aluminum           | 0.03                                                              | 0.030                 | 0.00037              |
|    | Copper             | 0.30                                                              | 0.031                 | 0.00038              |
|    | Gold               | 0.35                                                              | 0.031                 | 0.00039              |
|    | Fluorine           | 0.02                                                              | 0.040                 | 0.00047              |
|    | Bismuth            | 1.0 40-2.5                                                        | 0.023                 | 0.00040              |
| 20 | Antimony           | 1.0 20-1.5                                                        | 0.031                 | 0.00050              |
|    | Columbium          | 0.35                                                              | 0.019                 | 0.00023              |

<sup>1</sup> The range set forth is discussed below.

As previously mentioned, certain positive promoters may also be alloyed with the aforementioned lead-selenium base alloys and such promoters are listed in column 1 of Table IV. The second column of Table IV like the corresponding column of Table III sets forth the order of the maximum concentration limits by weight percent of such promoters to the base alloys effective for achieving the objects of the invention. Again it will be observed that concentrations of the positive promoters to the lead-selenium base alloys in amounts in excess of that contained in column 2 of Table IV have no appreciable effect in beneficially altering the electrical properties with which this invention is concerned, and in this sense the limits indicated are to be considered critical.

Column 3 of Table IV sets forth the minimum concentration by weight percent of the positive promoters listed affording useful heat pump elements of positive polarity.

40 Columns 4 and 5 set forth the Peltier E.M.F. and resistivity characteristics at room temperature of the alloy or composition resulting from the addition of the aforementioned positive promoters in the amount shown in column 2 after high temperature annealing as aforementioned.

Table IV

|    | Positive promoters | Order of maximum effective concentration limit by weight percent | Order of minimum effective concentration limit by weight percent | Peltier E.M.F., volts | Resistivity, ohm-cm. |
|----|--------------------|------------------------------------------------------------------|------------------------------------------------------------------|-----------------------|----------------------|
| 50 |                    |                                                                  |                                                                  |                       |                      |
|    | Sodium             | 0.08                                                             | 0.0025                                                           | +0.054                | 0.0019               |
|    | Potassium          | 0.15                                                             | 0.007                                                            | +0.075                | 0.0076               |

55 As aforementioned, the lead-selenium base alloy previously described is a two-phase alloy. When the aforementioned promoter additions are incorporated in the base alloy, such promoter additions become distributed between the two phases. We have discovered that the nature of such distribution has negligible effect on the electrical properties of the composition in all cases except that of bismuth and antimony. Accordingly, in the case of bismuth and antimony the maximum effective concentration is dependent upon the lead content of the lead-selenium base alloy within the ranges stated therefor as shown in Figure 3. We have found 2.5% by weight bismuth to be the maximum effective concentration for lead-selenium base alloys containing 73.5% lead; for base alloys containing less lead the maximum effective bismuth concentration is somewhat less, that is ranges down to 0.40% by weight when the lead content ranges down to 72.45%. Similarly, in the case of antimony, the maximum effective concentration is dependent upon the lead content of the lead-selenium base alloy within the

range stated therefor. We have found 1.5% by weight antimony to be the maximum effective concentration for lead-selenium base alloys containing 73.5% lead; for base alloys containing less lead the maximum effective antimony concentration is somewhat less, that is ranges down to 0.20% by weight when the lead content ranges down to 72.45%.

This behavior of bismuth and antimony is thought to be due to the formation of a bismuth-lead-selenium or an antimony-lead-selenium complex within the intergranular phase aforementioned which accounts for a portion of the addition. All other third element additions aforementioned, both positive and negative, form complexes with the second or intergranular phase aforementioned to a much lesser extent than do bismuth and antimony and for purposes of this invention, in the cases of such other additions these effects are inconsequential. Accordingly, no changes in the concentration limits thereof are necessary as the proportions of lead and selenium in the base alloy vary within the range stated therefor.

In Tables III and IV above, the Peltier E.M.F. and resistivity data given is in both cases for the 72.45% lead, balance substantially all selenium composition containing the promoter addition in question in the maximum effective amount indicated in the table (in the case of bismuth and antimony, the lower maximum effective amount indicated).

Table V below, first column thereof, lists the additions which we have found effective as negative promoters when added to the aforementioned lead-sulphur base alloys or compositions. The second column of Table V lists the order of the maximum concentration limits by weight percent of such promoters to the base alloys effective for achieving the objects of the invention. It is to be understood that these concentration limits are the maximum which effectively alter the electrical properties of the base alloy. Concentrations in excess of the stated amounts of such additives have no appreciable effect in beneficially altering the electrical properties with which this invention is concerned, and in this sense the limits indicated are to be considered critical. The third and fourth columns of Table V set forth the electrical properties at room temperature of lead-sulphur alloys promoted with the maximum useful concentrations of the negative promoters after high temperature annealing as hereinbefore described.

Table V

| Negative promoters | Order of maximum effective concentration limits by weight percent | Peltier E.M.F., volts | Resistivity, ohm-cm. |
|--------------------|-------------------------------------------------------------------|-----------------------|----------------------|
| Zirconium          | 0.40                                                              | 0.011                 | 0.00022              |
| Indium             | 0.50                                                              | 0.016                 | 0.00024              |
| Bromine            | 0.35                                                              | 0.016                 | 0.00024              |
| Chlorine           | 0.15                                                              | 0.016                 | 0.00025              |
| Titanium           | 0.20                                                              | 0.020                 | 0.00029              |
| Iodine             | 0.55                                                              | 0.030                 | 0.00042              |
| Tantalum           | 0.70                                                              | 0.030                 | 0.00042              |
| Bismuth            | 11.0-3.0                                                          | 0.035                 | 0.00061              |
| Antimony           | 1.0-50-3.0                                                        | 0.038                 | 0.00064              |
| Gallium            | 0.30                                                              | 0.035                 | 0.00058              |
| Columbium          | 0.40                                                              | 0.032                 | 0.00023              |
| Uranium            | 1.0                                                               | 0.030                 | 0.00024              |

<sup>1</sup> The range set forth is discussed below.

As previously mentioned, certain positive promoters may also be alloyed with the aforementioned lead-sulphur base alloys and such promoters are listed in column 5 of Table VI. The second column of Table VI like the corresponding column of Table V sets forth the order of the maximum concentration limits by weight percent of such promoters to the base alloys effective for achieving the objects of the invention. Again it will be observed that concentrations of the positive promoters to the lead-sulphur base alloys in amounts in excess of that contained in column 2 of Table V have no appreciable effect in bene-

ficially altering the electrical properties with which this invention is concerned, and in this sense the limits indicated are to be considered critical.

Column 3 of Table VI sets forth the minimum concentration by weight percent of the positive promoter listed affording useful heat pump elements of positive polarity. Columns 4 and 5 set forth the Peltier E.M.F. and resistivity characteristics at room temperature of the alloy or composition resulting from the addition of the aforementioned positive promoter in the amount shown in column 2 after high temperature annealing as aforementioned.

Table VI

| Positive promoters | Order of maximum effective concentration limit by weight percent | Order of minimum effective concentration limit by weight percent | Peltier E.M.F., volts | Resistivity, ohm-cm. |
|--------------------|------------------------------------------------------------------|------------------------------------------------------------------|-----------------------|----------------------|
| Silver             | 2.0                                                              | 0.70                                                             | 0.081                 | 0.020                |

As aforementioned, the lead-sulphur base alloy previously described is a two-phase alloy. When the aforementioned promoter additions are incorporated in the base alloy, such promoter additions become distributed between the two phases. We have discovered that the nature of such distribution has negligible effect on the electrical properties of the composition in all cases except that of bismuth and antimony. Accordingly, in the case of bismuth and antimony the maximum effective concentration is dependent upon the lead content of the lead-sulphur base alloy within the ranges stated therefor as shown in Figure 3. We have found 3.0% by weight bismuth to be the maximum effective concentration for lead-sulphur base alloys containing 87.10% lead; for base alloys containing less lead the maximum effective bismuth concentration is somewhat less, that is ranges down to 1.0% by weight when the lead content ranges down to 86.63%. Similarly, in the case of antimony, the maximum effective concentration is dependent upon the lead content of the lead-sulphur base alloy within the range stated therefor. We have found 3.0% by weight antimony to be the maximum effective concentration for lead-sulphur base alloys containing 87.10% lead; for base alloys containing less lead the maximum effective antimony concentration is somewhat less, that is ranges down to 0.50% by weight when the lead content ranges down to 86.63%.

This behavior of bismuth and antimony is thought to be due to the formation of a bismuth-lead-sulphur or an antimony-lead-sulphur complex within the intergranular phase aforementioned which accounts for a portion of the addition. All other third element additions aforementioned, both positive and negative, form complexes with the second or intergranular phase aforementioned to a much lesser extent than do bismuth and antimony and for purposes of this invention, in the cases of such other additions these effects are inconsequential. Accordingly, no changes in the concentration limits thereof are necessary as the proportions of lead and sulphur in the base alloy vary within the range stated therefor.

In Tables V and VI above, the Peltier E.M.F. and resistivity data given is in both cases for 86.63% lead, balance substantially all sulphur composition containing the promoter addition in question in the maximum effective amount indicated in the table (in the case of bismuth and antimony, the lower maximum effective amount indicated).

From the foregoing description, it will be noted that the maximum concentrations of beneficial impurity for promoted terminal compositions vary from 4.22% by weight (i.e. 3.02% excess lead plus 1.20% maximum for any promoter) in the case of the terminal lead-tellurium composition, to 6.6% by weight (i.e. 4.1% excess lead plus 2.5% maximum for any promoter) in the case of

the terminal lead-selenium composition, to 6.9% by weight (i.e. 3.9% excess lead plus 3.0% maximum for any promoter) in the case of the terminal lead-sulphur composition. Thus, the maximum amount of beneficial impurity for any promoted composition is 6.9% by weight. While, as aforescribed, the maximum amount of beneficial impurity for any unpromoted composition is 10.4% by weight. Accordingly, it can be said that the maximum amount of beneficial impurity for any composition aforescribed is, in round numbers, about 10% by weight.

Typical data of the aforescribed compositions are, by way of example, shown in Figures 5 and 5a wherein the Peltier E.M.F. in volts (left-hand scale) and

$$\frac{\pi^2}{\rho}$$

in watts per centimeter (right-hand scale) are plotted against the log of the resistivity in ohm-centimeter.

In Figure 5 curves G, H and I represent compositions consisting essentially of lead and tellurium, lead and selenium, and lead and sulphur, respectively, within the ranges aforesigned, and which curves graphically illustrate variation in the relationship between Peltier coefficient ( $\pi$ ) and resistivity ( $\rho$ ) with additions of negative promoters to the respective base compositions (the right-hand ends of such curves representing the base compositions). Similarly, curves J, K and L represent compositions consisting essentially of lead and tellurium, lead and selenium, and lead and sulphur, respectively, within the ranges aforesigned, and which curves graphically illustrate variations in the value of the quotient

$$\frac{\pi^2}{\rho}$$

with additions of negative promoters to the base composition (the right-hand ends of such curves representing the base compositions).

In Figure 5a curves M, N and O represent compositions consisting essentially of lead and tellurium, lead and selenium, and lead and sulphur, respectively, within the ranges aforesigned, and which curves graphically illustrate variation in the relationship between Peltier coefficient ( $\pi$ ) and resistivity ( $\rho$ ) with additions of positive promoters to the respective base compositions (the right-hand ends of such curves representing the minimum effective concentration of positive promoters aforescribed). Similarly, curves P, Q and R represent compositions consisting essentially of lead and tellurium, lead and selenium, and lead and sulphur, respectively, within the ranges aforesigned, and which curves graphically illustrate variation in the value of the quotient

$$\frac{\pi^2}{\rho}$$

with additions of positive promoters to the base composition (the right-hand ends of such curves representing the minimum effective concentration of positive promoters aforescribed).

In Figures 5 and 5a curves J, K, L and P exhibit maximum values of the quotient

$$\frac{\pi^2}{\rho}$$

The curves Q and R exhibit extremal values for the maximum concentration of positive promoter. The resistivity of the right-hand coordinate of Figures 5 and 5a (0.1 ohm-cm.) is characteristic of semi-conductor materials. The resistivity of the left-hand coordinate of Figures 5 and 5a (0.0001 ohm-cm.) is characteristic of a metal. The maximum and extremal values aforesigned occur at values of Peltier coefficient and resistivity intermediate to those of metals and semi-conductors. More-

over, as aforesigned, semi-metallic elements embodying the present invention exhibit low thermal conductivity approaching that of a semi-conductor. High values of the quotient

$$\frac{\pi^2}{\rho}$$

and simultaneously the low values of thermal conductivity (K) afford the high performance factors desired for heat pump elements.

Further illustrative data for some of the compositions aforesigned are shown by way of example in Figure 6 wherein the left-hand scale is in terms of the performance coefficient (refrigeration)

15

$$\frac{Q_a}{EI} = \frac{Q_a}{Q_b - Q_a}$$

The right-hand scale is in terms of  $Q_a$  (the pumping rate) in watts, both plotted against the horizontal scale of current density, amp./cm.<sup>2</sup>. In Figure 6 curve S is a representative performance coefficient curve for compositions consisting essentially of lead and tellurium while curve T is a representative curve of the pumping rate ( $Q_a$ ) for the same compositions. Similarly, curve U is a representative performance coefficient curve for compositions consisting essentially of lead and sulphur, while curve V is a representative pumping rate curve ( $Q_a$ ) for the same compositions. From Figures 5 and 5a it will be readily ascertained that representative curves for compositions consisting essentially of lead and selenium will fall somewhat intermediate the curves in Figure 6 for the lead and tellurium and lead and sulphur compositions, respectively.

As will be apparent to those skilled in the art, all of the semi-metallic compositions aforesigned exemplary of the thermoelectric heat pump elements comprising binary metallic compounds and ternary compositions or alloys thereof having semiconductor-like conductivity afford heat pump characteristics of sufficient magnitude for practical application. By way of example, data is given in Table VII below illustrating such improved heat pumping characteristics.

In Table VII the first column in terms of composition and percent by weight lists various examples of compositions of the class described; the second column indicates the Peltier E.M.F. in volts dérivable from each of such compositions; the third column lists for each of such compositions the thermal conductivity in watts per centimeter degrees Centigrade; the fourth column lists for each of such compositions their resistivity in ohm-cm.; and the fifth column indicates for each of such compositions the performance factor thereof. It will be noted that the examples of compositions given include examples of each of the base alloys and at least one example of each of the base alloys to which a promoter has been added.

Table VII

| Composition, percent by weight | Peltier E.M.F., volts | Thermal conductivity, watts/cm., °C. | Electrical resistivity, ohm-cm. | Performance factor, $\pi^2/2K_a$ , degrees C. |
|--------------------------------|-----------------------|--------------------------------------|---------------------------------|-----------------------------------------------|
| 62% Pb-38% Te                  | -0.126                | 0.022                                | 0.016                           | 22.7                                          |
| 62% Pb-38% Te +0.0027% Zr      | -0.105                | 0.025                                | 0.0026                          | 84.3                                          |
| 62% Pb-38% Te +0.0021% Na      | +0.088                | 0.025                                | 0.0022                          | 170.5                                         |
| 73% Pb-27% Se                  | -0.077                | 0.034                                | 0.0022                          | 40.9                                          |
| 73% Pb-27% Se +0.0017% Ti      | -0.073                | 0.037                                | 0.0012                          | 57.5                                          |
| 73% Pb-27% Se +0.06% Na        | +0.054                | 0.035                                | 0.0019                          | 122.0                                         |
| 87% Pb-13% S                   | -0.070                | 0.036                                | 0.0027                          | 25.5                                          |
| 86.7% Pb-13.3% S +0.02% In     | -0.054                | 0.040                                | 0.0010                          | 35.8                                          |
| 86.7% Pb-13.3% S +2.0% Ag      | +0.083                | 0.033                                | 0.0130                          | 18.1                                          |

<sup>1</sup> Positive.

Referring to Table VII, a comparison of the performance factor column indicates that the promoted alloys afford better pumping characteristics than the base alloys. This conclusion can be justified by reference to Table VIII below containing actual pumping data on a bismuth promoted lead-tellurium alloy by way of example.

Table VIII

| Composition                                   | Performance factor (calculated, $\pi^2(2K_p)$ , C.) | Current density, amp./cm. <sup>2</sup> | Temp. diff., °C. | Heat pump rate, watts | Performance coefficient (refrigeration) |
|-----------------------------------------------|-----------------------------------------------------|----------------------------------------|------------------|-----------------------|-----------------------------------------|
| 62% Pb-38% Te (negative polarity).            | 63                                                  | 1.58                                   | 1.7              | 0.002                 | 5.0                                     |
|                                               |                                                     | 3.15                                   | 3.2              | 0.005                 | 1.6                                     |
|                                               |                                                     | 6.30                                   | 5.9              | 0.01                  | 0.85                                    |
|                                               |                                                     | 12.6                                   | 9.7              | 0.03                  | 0.42                                    |
| 62% Pb-38% Te + 0.05% Bi (negative polarity). | 80                                                  | 1.58                                   | 1.3              | 0.0007                | 14.3                                    |
|                                               |                                                     | 3.15                                   | 2.2              | 0.016                 | 5.4                                     |
|                                               |                                                     | 6.30                                   | 4.8              | 0.035                 | 2.8                                     |
|                                               |                                                     | 12.6                                   | 8.1              | 0.075                 | 1.3                                     |
| 62% Pb-38% Te + 0.10% Bi (negative polarity). | 81                                                  | 1.58                                   | 1.3              | 0.01                  | 17.0                                    |
|                                               |                                                     | 3.15                                   | 2.2              | 0.02                  | 8.4                                     |
|                                               |                                                     | 6.30                                   | 4.6              | 0.05                  | 3.1                                     |
|                                               |                                                     | 12.6                                   | 7.8              | 0.10                  | 2.1                                     |

The data of Table VIII shows that the performance coefficient and heat pumping rate increase as the bismuth concentration is increased. Similar effect can be observed in connection with other of the base alloys and with other promoters of the given base alloys. It will be noted also that for a given composition and current density, the induced temperature difference and heat pumping rate are related. As one is increased the other is decreased. In the range shown, the induced temperature difference and heat pumping rate increase with increased current density while the performance coefficient decreases. Since it is usually desirable to have most of these parameters as high as possible, there is no particular optimum current density; instead the current density is a parameter to be chosen according to the application involved.

Table VIII above gives typical data for all of the aforementioned compositions applicable equally to thermoelectric heat pump elements of positive as well as negative polarity. By way of example Table IX following gives heat pumping data for a specific thermoelectric heat pump element of positive polarity.

Table IX

| Composition                                  | Current density, amp./cm. <sup>2</sup> | Temp. diff., °C. | Heat pump rate, watts | Performance coefficient (refrigeration) |
|----------------------------------------------|----------------------------------------|------------------|-----------------------|-----------------------------------------|
| 62% Pb-38% Te + 0.2% Tl (positive polarity). | 3.15                                   | 1.3              | 0.015                 | 3.7                                     |
|                                              |                                        | 6.30             | 2.6                   | 0.031                                   |
|                                              |                                        | 12.6             | 4.6                   | 0.061                                   |
|                                              |                                        | 25.2             | 4.8                   | 0.122                                   |

With a single element heat pump of the type shown schematically in Figure 1 a temperature suppression at the cooling junction of 25° C. has been attained, and a temperature elevation at the heating junction of at least 100° C. has been attained. Similarly, as indicated in Tables VIII and IX, a performance coefficient of cooling as high as 17 can be attained. In fact, referring to Figure 6, it will be observed that as the current density approaches smaller values the performance coefficient rises steeply indicating that even higher performance coefficients can be attained at lower current densities. As aforementioned, similar performance coefficients can be attained at the heating junction since the performance coefficient for heating is the performance coefficient for cooling plus one. Moreover, as will also be apparent from Figure 6, pumping rates approaching .2 of a watt

for a single unit of a quarter inch diameter at a current density in excess of 25 amperes per square centimeter are attainable. Since the pumping rate increases as the performance coefficient decreases the current density for a practical application should be chosen to give simultaneously the highest possible values of performance coefficient and pumping rate according to the nature of the application.

We have further found that suitable additional positive thermoelectric elements exhibiting positive electrical characteristics as previously defined, and useful for heat pumping may comprise lead and tellurium in which there is an excess of tellurium over and above the amount thereof necessary for satisfying the stoichiometric portions of the compound lead-telluride. Such additional alloys or compositions may contain added beneficial impurity substances, and such substances, as before, are also denominated hereinafter as "positive promoters." These additional alloys or compositions may also be characterized as binary metallic compounds of slightly imperfect composition by reason of the excess of tellurium over lead and/or containing added beneficial impurity substances. Such additional alloys or compositions, as previously related, may be termed semi-metallic alloys or compositions, and have semiconductor-like conductance, (both electrical and thermal), similarly to the binary and ternary alloys already discussed.

More specifically, we have found especially useful for thermoelectric elements exhibiting positive electrical characteristics, base alloys or compositions consisting essentially of lead and tellurium in which lead is present in the range of from 58.0% to 61.8% by weight and the balance in the range of from 42.0% to 38.2% by weight tellurium.

The portions of the lead and tellurium constituents as last set forth must be considered critical if the compositions are to have the electrical properties desired in heat pumps.

As before, not only is the range last described of the tellurium rich lead-tellurium base compositions considered to be critical but so also is the purity. Again, the limit of tolerable metallic impurity in the final composition has been found to be on the order of 0.01% and the composition must be substantially oxygen free if the mechanical and electrical properties desired are to be obtained and be reproducible. Such purity may be achieved in the manner already described in the fabrication of the aforementioned lead and tellurium, selenium and sulphur compositions containing an excess of lead. An essential difference in the method of making the alloys of the last noted tellurium rich lead-tellurium compositions resides in the rate of cooling after annealing. In this regard, we have found a cooling rate of 50° C. per hour to be sufficiently low to provide the element with adequate mechanical strength.

The tellurium rich base lead-tellurium alloys, as in the case of the first described alloys, may also be described metallographically as a two-phase alloy. The excess of tellurium in the tellurium rich compositions behaves much as the excess of lead in the first discussed alloys in that it controls the polarity of the conductivity and thermoelectric power in the primary lead-telluride phase, and it also forms a detectable second phase at the grain boundaries as already above discussed. The compositions are further adequately stable for temperature applications ranging up to 400° C.

It is to be observed from the foregoing that the tellurium rich base lead-tellurium compositions contain from 38.20% to 42.0% by weight tellurium, or from 0.14% to 6.7% by weight tellurium of the total composition over and above the tellurium stoichiometrically necessary to combine with the lead.

The excesses of tellurium aforementioned in the compositions last described may be denominated impurities with respect to the primary lead-telluride phase. Such

impurities, as before, must be distinguished from any undesired impurities as previously discussed. Accordingly, and as before, for purposes of this specification and the appended claims, such excess tellurium amounts purposely present in the composition are denominated "beneficial impurities." Likewise, it is the presence of such beneficial impurities that affords these last mentioned additional compositions their desired electrical characteristics and distinguish such semi-metallic alloys or compositions of the invention from the primary phase intermetallic compound lead-telluride. Such beneficial impurities afford the intermetallic compounds lead-telluride a lower resistivity without proportional sacrifice of Peltier E.M.F. or low thermal conductivity and results in a composition having what may be termed semiconductor-like electrical conductance or conductivity. It should be noted that such excess tellurium induces in the compositions aforescribed a Peltier E.M.F. of positive polarity and positive conductivity, thereby affording a thermoelectric heat pump element having utility in the manner already described.

We have further discovered that the electrical characteristics of thermoelectric elements for heat pumps of the last mentioned range of excess tellurium impurity (again for convenience hereinafter denominated "base compositions") can be markedly and advantageously altered in a reproducible manner by the addition thereto of controlled amounts of matter other than the constituents of such base compositions. Such additions are also here denominated "beneficial impurities" as distinguished from undesired impurities as previously discussed. Again, such additions are denominated "promoters" since, as will hereinafter appear, they tend to enhance the electrical characteristics desired in thermoelectric heat pump elements of the last mentioned base composition. As before, the amounts of such promoters in terms of percent by weight of the base composition are very small, and for such promoters to be most effective and afford reproducibility of electrical properties the base composition to which they are added should be of even greater purity, i.e. containing even less of undesired and uncontrolled impurities. As a practical matter, we have found that the tellurium rich base lead-tellurium compositions should be of such purity in this regard as to contain not in excess of 0.001% by weight undesired impurity. Similarly to the first disclosed promoted compositions the lead content of the instant base composition should be in the range of from 59.0% to 61.8% lead by weight as against the range of lead of from 58.0% to 61.8% by weight above disclosed for the unpromoted compositions.

As already observed, the aforementioned base compositions of tellurium rich lead-tellurium compositions exhibit positive Peltier E.M.F. and positive conductivity. By the addition of the promoters to be hereinafter described, such positive electrical properties may be enhanced by the addition of certain promoters and such positive promoters in connection with the last mentioned base alloy effect an increase in the conductivity of the alloy and slight decrease in the Peltier E.M.F. Table X below, first column thereof, lists the additions which we have found effective as positive promoters when added to the last mentioned tellurium rich lead-tellurium base compositions. The second column of Table X lists the order of the maximum effective concentration limits by weight percent of such promoters to the base alloy effective for achieving the objects of the invention. It is understood that these concentration limits are the maximum which effectively alter the electrical properties of the noted base alloy. Concentrations in excess of the stated amounts of such additives have no appreciable effect in beneficially altering the electrical properties with which this invention is concerned, and in this sense the limits indicated are to be considered critical. The third and fourth columns of Table X set forth the electrical

properties at room temperature of the aforementioned tellurium rich lead-tellurium base compositions promoted with the maximum useful concentrations of the positive promoters after annealing.

Table X

| Positive promoters | Order of maximum effective concentration limits by weight percent | Peltier E.M.F., volts | Resistivity, ohm-cm. |
|--------------------|-------------------------------------------------------------------|-----------------------|----------------------|
| Sodium.....        | 0.14                                                              | 0.020                 | 0.00033              |
| Potassium.....     | 0.23                                                              | 0.027                 | 0.00037              |
| Thallium.....      | 0.60                                                              | 0.041                 | 0.0013               |

From the foregoing description it will be noted that the maximum concentrations of beneficial impurity for the last disclosed promoted tellurium rich lead-tellurium compositions varies from a minimum of 0.28% by weight (i.e., 0.14% by weight excess tellurium plus 0.14% by weight sodium) to 5.5% by weight (i.e. 4.9% by weight excess tellurium plus 0.60% by weight thallium), which fall well within the aforementioned maximum amount of beneficial impurity of about 10% by weight.

Typical data of the last aforescribed compositions is shown by way of example in Figure 7, which is similar to Figures 5 and 5a, wherein the Peltier E.M.F. in volts (left-hand scale) and

$$\frac{\pi^2}{\rho}$$

in watts per centimeter (right-hand scale) are plotted against the resistivity in ohm-centimeter.

In Figure 7, curve X represents compositions of tellurium rich lead-tellurium within the range afore-indicated and which curve graphically illustrates variations in the relationship between Peltier coefficient ( $\pi$ ) and resistivity ( $\rho$ ) with addition of positive promoters to the last noted base compositions (the right-hand end of such curve representing the minimum effective concentration of positive promoters last described). Similarly, curve W represents the last aforementioned tellurium rich lead-tellurium compositions within the range afore-indicated and which curve graphically illustrates variations in the value of the quotient

$$\frac{\pi^2}{\rho}$$

with additions of positive promoters to the base composition last discussed (the right-hand end of such curve representing the minimum effective concentration of positive promoters last described). The curve W exhibits maximum values of the quotient

$$\frac{\pi^2}{\rho}$$

The resistivity of the right-hand coordinate of Figure 7 (0.1 ohm-cm.) is characteristic of semiconductor materials. The resistivity of the left-hand coordinate of Figure 7 (0.0001 ohm-cm.) is characteristic of a metal. The maximum and extremal values aforementioned occur at values of Peltier coefficient and resistivity intermediate to those of metals and semiconductors. Moreover, as previously mentioned, semi-metallic elements embodying the present invention exhibit low thermal conductivity approaching that of a semiconductor. High values of the quotient

$$\frac{\pi^2}{\rho}$$

and simultaneously the low values of thermal conductivity ( $K$ ) afford the high performance effect desired for heat pump elements.

In Table XI below, the first column in terms of composition and percent by weight, lists various examples of

compositions of the class last described; the second column indicates the Peltier E.M.F. in volts derivable from each of such compositions; the third column lists for each of such compositions the thermal conductivity in watts per centimeter degrees centigrade; the fourth column lists for each of such compositions the resistivity in ohm-cm.; and the fifth column indicates for each of such compositions the performance factor thereof. It will be noted that the examples of compositions given include tellurium rich lead-tellurium base alloys and including each of the positive promoters last discussed.

Table XI

| Composition, percent by weight | Peltier E.M.F., volts | Thermal conductivity, watts/cm., °C. | Electrical resistivity, ohm-cm. | Performance factor, $\pi^2/2K_P$ , degrees C. |
|--------------------------------|-----------------------|--------------------------------------|---------------------------------|-----------------------------------------------|
| 61.7% Pb+38.3% Te+0.007% Na    | 0.0625                | 0.030                                | 0.00135                         | 48.3                                          |
| 61.7% Pb+38.3% Te+0.012% K     | 0.062                 | 0.030                                | 0.00155                         | 41.3                                          |
| 61.7% Pb+38.3% Te+0.18% Ti     | 0.042                 | 0.030                                | 0.00135                         | 21.8                                          |

We claim:

1. A thermoelectric heat pump comprising, at least a pair of thermoelectrically dissimilar electrical conductors joined in circuit to provide at least a pair of thermoelectric junctions, at least one of said conductors being a semi-metallic element selected from the class of binary and ternary alloys of slightly imperfect stoichiometric composition and having semiconductor-like conductivity, said semi-metallic element affording transfer of heat therethrough when said circuit is energized, thereby effecting cooling at one of said junctions and heating at the other of said junctions.
2. A thermoelectric heat pump according to claim 1 in which the imperfection of composition of said semi-metallic element comprises a departure from stoichiometry of said alloy by an amount not in excess of 10.4 percent by weight of said alloy.
3. A thermoelectric heat pump according to claim 1 in which the imperfection of composition of said semi-metallic element comprises a stoichiometric excess of one of the constituents.

4. A cold producing thermoelement comprising two circuit members of different respective materials, a heat absorbing element having good heat conductivity and slight thermoelectric power conductively joined intermediate said members to form together therewith a thermoelectric junction, at least one of said two members consisting of a binary compound of two metals of a slightly imperfect composition departing from perfect stoichiometry by an amount of at most 2 percent by weight of the total material of said member, and having semiconductor-like electric conductance.

5. In a thermoelement according to claim 4, said amount consisting of an excess of one of the two metals over the other.

6. A cold producing thermoelement, comprising two circuit members of different metallic materials, heat absorbing element having good heat conductivity and slight thermoelectric power of large differential thermoelectric power, and an intermediate part of larger conductance and of negligible differential thermoelectric power as compared with said two members, said members and said part being joined together to form a thermoelectric junction, at least one of said members consisting of a binary compound of two metals of a slightly imperfect composition departing from perfect stoichiometry by an amount of at most 2 percent by weight of the total mate-

rial of said member and having semiconductor-like electric conductance.

7. A cold producing thermoelement, comprising two circuit members of different metallic materials, and an intermediate part of larger conductance and of negligible differential thermoelectric power as compared with said two members, said members and said part being joined together to form a thermoelectric junction, at least one of said members consisting of a binary compound of two metals of a slightly imperfect composition departing from perfect stoichiometry by an amount of at most 2 percent by weight of the total material of said member and having semiconductor-like electrical conductance.

8. A thermoelectric heat pump comprising a pair of circuit members joined in circuit to provide a thermoelectric junction, at least one of said two members consisting of a binary compound of two metals in which there is a departure from perfect stoichiometry by an amount not in excess of 10.4% by weight of said one member and having semiconductor-like electric conductance.

9. A thermoelectric heat pump comprising a pair of circuit members joined in circuit to provide a thermoelectric junction, at least one of said two members consisting of a binary compound of two metals in which there is a departure from perfect stoichiometry consisting of an excess of one of the two metals over the other by an amount not in excess of 10.4% by weight of said one member and having semiconductor-like conductance.

10. A thermoelectric heat pump comprising a pair of circuit members joined in circuit to provide a thermoelectric junction, at least one of said two members consisting of a binary compound of two elements in which there is a departure from perfect stoichiometry consisting of a stoichiometric excess of one of said elements over the other of said elements and a beneficial impurity substance not in excess of 6.9% by weight of said one member and having semiconductor-like conductance.

11. A thermoelectric heat pump comprising a pair of circuit members joined in circuit to provide a thermoelectric junction, at least one of said two members being a semi-metallic element from the class of binary and ternary alloys of metals in which there is a departure from perfect stoichiometry by an amount not in excess of 10.4% by weight of said one member and having semiconductor-like conductance.

12. A thermoelectric heat pump comprising a pair of circuit members joined in circuit to provide a thermoelectric junction, at least one of said two members being a semi-metallic element from the class of binary and ternary alloys of metals of imperfect composition in which there is a departure from perfect stoichiometry consisting of an excess of one of the metals of an amount not in excess of 10.4% by weight of said one member and having semiconductor-like conductance.

13. A thermoelectric heat pump comprising a pair of circuit members joined in circuit to provide a thermoelectric junction, at least one of said two members being a semi-metallic composition from the class of binary and ternary alloys of elements of imperfect composition in which there is a departure from perfect stoichiometry consisting of a stoichiometric excess of at least one of said elements and a beneficial impurity substance not in excess of 6.9% by weight of said one member and having semiconductor-like conductance.

References Cited in the file of this patent

UNITED STATES PATENTS

- 2,811,440 Fritts et al. \_\_\_\_\_ Oct. 29, 1957  
2,811,571 Fritts et al. \_\_\_\_\_ Oct. 29, 1957

UNITED STATES PATENT OFFICE  
CERTIFICATE OF CORRECTION

Patent No. 2,896,005

July 21, 1959

Robert W. Fritts et al.

It is hereby certified that error appears in the printed specification of the above numbered patent requiring correction and that the said Letters Patent should read as corrected below.

Column 6, line 42, for "sulphur of" read -- sulphur or --; column 8, line 59, for "electrial" read -- electrical --; line 64, for "and/reducing" read -- and/or reducing --; column 12, Table I, heading to second column, last line thereof, for "percent, 0.80" read -- percent --; same table, same second column, last line opposite "Uranium" strike out the leaders and insert instead -- 0.80 --; third column, heading thereto, for "Peltier E.M.F., volts, 0.022" read -- Peltier E.M.F. volts --; same column, last line, strike out the leaders and insert instead -- 0.022 --; same table I, fourth column, heading thereto, for "Resistivity, ohm-cm., 0.00020" read -- Resistivity, ohm-cm. --; same table I, same fourth column, last line, strike out the leaders and insert instead -- 0.00020 --; column 13, line 75, for "hereinbfone" read -- hereinbefore --.

Signed and sealed this 21st day of June 1960.

(SEAL)

Attest:

KARL H. AXLINE

Attesting Officer

ROBERT C. WATSON  
Commissioner of Patent